# EUROPEAN PATENT SPECIFICATION

(11) **EP 0 064 309 B1**
(45) Date of publication and mention of the grant of the patent: **04.02.1987**
(21) Application number: 82200472.7
(22) Date of filing: 20.04.1982
(51) Int. Cl.: D21H 3/18, D21H 3/02, D21H 5/14

(54) **A process for the manufacturing of paper, particularly corrugated paperboard**
Ein Verfahren zur Herstellung von Papier, insbesondere Wellenpappe
Un procédé de fabrication de papier, en particulier du carton ondulé

(30) Priority: 05.05.1981 IT 2151281
(43) Date of publication of application: 10.11.1982
(73) Proprietor: Industrial Financial Development S.r.l., I-03032 Arce (FR)
(72) Inventor: Mortarotti, Emilio, I Alessandria (IT)
(74) Representative: Dragotti, Gianfranco

## Description

The present invention relates to a process forthe manufacturing of paper, particularly of paper useful as the intermediate layer ("medium") of corrugated paper board, and to the thus resulting product.

It is known that the corrugated paper boards in their simplestform, consist of three layers, namely two outer layers, forming the faces of the paper board and called "liners", and an intermediate, corrugated layer known in the related art as the "medium".

In the case of the five layer corrugated paper boards, there are provided two layers of corrugated "medium" paper, each one being interposed between two layers of "liner".

It is also known that, owing to the main use of the corrugated paper boards in the packing field the most significant properties of the single component layers, for an evaluation as a whole of the corrugated paper boards are the crushing strength (also known as the "Concora"), the water repellence and the wet strength.

In the past the "medium" papers were manufactured from straw, but such a technology is being almost worldwide abandoned, both because the straw handling costs became too much heavy, (particularly with respect to the transportation and the involved labour) and owing to the pollution problems of the industrial effluents deriving from such a raw material.

Presently the "medium" papers are produced according to technologies which can be essentially referred to two classes of raw materials:
a) "medium" paper produced from mixtures of particles or chips or wood cooked by chemical processes (80%) and waste paper (20%); these papers are also called "semichemical" papers (or papers from semichemical pulp and are increasingly expensive due to the prevalence of a valuable material such as the wood.
b) "medium" papers produced from mixtures of waste paper which are then improved by surface treatment of the resulting paper with starches or resins, the so-called "flutings" being thus obtained.

In this case too, apart from the lower quality of the resulting paper, the manufacturing costs are increased not so mainly due to the raw material being used, but owing to the additional operations required.

It is enough to observe that the starch is added to the paper in the already substantially dried condition, as coming out of the drying section, in form of a thin surface layer, applied with a water solution having a concentration of about 2%, whereby the treated paper must be thereafter dried again with a relevant energy consumption.

Lastly it is worth to note that generally in the paper industry the effluent waters resulting from the attack of the wood particles (also known as the "black liquors") constitute a very serious problem from the point of view of the pollution and their treatment heavily affects the manufacturing costs.

In the US-A-3305435 a method is disclosed for making paper stiffened with waste pulp liquor solids, according to which the sheet of paper stock, either after drainage and drying or during the drying, is treates with waste pulp liquor having a solid content of 5 to 25%, preferably 15%.

In the CH-A-450891 a method is disclosed in which black liquors are added eitherto the starting suspension of fibres or to the sheet being formed, orto the already completed sheet, the black liquors being beforehand treated so as to bring the pH to a value higher than the neutral value, so as to precipitate their solid content.

The main purpose of the present invention is that of providing a process for the manufacturing of paper, particularly "medium" paper for corrugated paper board, which permit less valuable raw material to be used, the properties of crush resistance and water repellency being maintained at the same level or, the type and concentration of raw materials being the same, permits the afore said properties to be improved.

A more specific purpose of the present invention is that of providing a process of the afore said type which, in the case of the "semichemical" papers, and the physical and mechanical properties being the same particularly the crush strength being the same, permits the contents of wood pulp to be reduced.

Another likely more specific purpose of the present invention is that of providing a process of the afore said type which in the case of "fluting" paper, permits the crush strength to be increased by about 20%.

A further purpose of the present invention is that of providing a process for the manufacturing of improved paper products, such as cardboards, wherein the "stiffness" it is a qualitatively impor- tantfeature. These and other purposes are fulfilled by a process for making paper, cardboards or paperboards, from a fibre suspension, wherein a paper having a moisture content not greater than 50% is treated with black liquor, characterized in that the black liquor has a solid content from 10% to 50%, the fibres contain at least 20% of waste paper fibres, and the black liquor is added with polyvinyl alcohol.

It has been in fact found that the property of the black liquors of improving the properties of the treated paper is thus enhanced.

According to a further embodiment of the invention, when the black liquors are to be used for the treatment of coloured papers, even of light colours, they can be previously treated by partial whitening and subsequent dyeing (for instance by means of H₂0₂) in a per se known manner.

It has been in fact surprisingly found that the black liquors, which to date had no use or had a limited use in different technical fields and were only a problem from the point of view of the depuration of the effluent waters of paper manufacturing industries, when are applied as a thin layer to the paper being dried, provided that they are previously concentrated to a contents of 10 to 50% of dry material, preferably of 30 to 50%, permit the following results to be achieved:
1) In the case of the semichemical papers, (80% of wood pulps and 20% of waste paper pulp), the crush strength (Concora) is increased by more than 20% whereby the use of semichemical paper of lower grams per square meter is permitted to obtain corrugated paperboard having the same crushing strength.
2) Alternatively, in the case of the semichemical papers, the ratio between wood pulp and waste paper pulp can be changed, passing for instance from 80:20 to 60:40, the physical and chemical properties, particularly the crushing strength, being maintained unvaried. The economical advantage is self-evident, if attention is paid to the fact that by the waste paper pulp an economy of 30 to 50% with respect to the wood pulp is achieved.
3) In the case of the "fluting" papers, wherein to date the necessary crushing strength is obtained by applying starch or resins, there is not only achieved a saving of energy (in the previously stated sense) and of raw materials, since starches and resins are more expensive than the black liquors, but also better results are obtained as regards the increase of the crushing strength. In this specific embodiment it is preferable that the concentration of the black liquors is higher, of the order of 40 to 50%.
4) In the case of paper products in which the "stiffness" effect is important as regards the quality and thus the price of the product, (as for instance cardboards for industrial packings, or the non white layers therefor an improved product can be obtained at a lower cost.
5) By the process of the invention there are again industrially acceptable the plants for the manufacturing of paper and cellulose from straw, since the problem of the effluent and of the realted pollution is advantageously solved.

Several attempts have been made in the past in order to reuse or recycle the black liquors, those attempts only involving the addition of the black liquors to the aqueous suspension of fibres before the forming of the paper sheet without any previous concentration step: these attempts were essentially useless since, although an increase of grams per square meter occurred, the physical and mechanical properties of the resulting paper got worse.

On the contrary, the qualifying and fully surprising feature, besides being novel, of the process of the invention is that by coating the paper, already dried to an optimum value of residual moisture content, with the black liquors, also previously concentrated, the resulting product is qualitatively and relevantly improved.

In this connection, the field tests demonstrated that a difference of the moisture content of 20 to 30% is recommended to ensure the desired results: otherwise stated, if the residual moisture content of the paper is about 30% it will be enough that the black liquors are concentrated to not more than 50% to obtain the optimum results.

Without imposing undue limitations to the present invention it seems plausible the hypothesis according to which the black liquors, owing to the concentration step, acquire the faculty of crystallizing and polimerizing (depending on the nature of the components), onto the surface of the paper being treated, thus giving place to the already mentioned "stiffness" effect, like or more than the traditional treatment agents, but with the previously mentioned advantages.

In this connection it seems reasonable to suppose that the better results, as obtained with the black liquors, can be attributed to a greater compatibility with the fiber substances which are treated therewith.

For the preparation of the black liquors to be used for the present invention there is carried out the washing and squeezing of the wood particles or chips after the chemical cooling the operation being repeated the most suitable number of times; like treatment is carried out on the pulp obtained from the beating operation as effected on the aforesaid chips, the resulting black liquors being recovered and combined.

As the black liquors useful for the present invention there are contemplated not only those resulting from semichemical and chemical cooking treatments of annual or multiannual plants, as by-products of the paper and/or cellulose manufacturing, but also the black liquors which are purposely produced from plants or wastes of annual and multiannual plants (such as straws of various nature, canes, etc.) saw mill wastes, vine- shoots, sawdusts and generally wood flours.

In the latter case these raw materials are chemically attacked with either acid or basic solutions, the chemical attack being effected to get the maximum yield of black liquors, whereas cellulose or hemicellulose, useful too in the paper industry, are obtained as the by-products.

The black liquors are then passed to a concentration plant, comprising two or more stages (depending on the sought concentration degree).

Clearly, the higher is the resulting concentration, the more economical is the use of the resulting black liquors, since the energy consumption for the drying of the treated paper will be lower.

Especially when "fluting" papers are to be treated, it is convenient to bring the concentration of the black liquors to values of 40 to 50%.

The black liquors, as it is evident, are produced in the plants for the manufacturing of chemical or semichemical paper starting from wood.

They can be used again in the same paper mill or even used in paper mills producing "fluting" paper, namely from waste paper pulp. In the latter case, of course, the concentration of the black liquors is brought to at least 35 to 40% for transport saving.

The resulting black liquors, having greater or lesser viscosity and consistence, depending on the concentration degree, are coated onto the paper during its drying step, by means of coating rollers, or of any other suitable device depending on the type of black liquors.

The coating of the paper can take place onto one or borh surfaces, or between one sheet and the other in the case of doubled paper, cardboard or paperboard, by using known coupling, coaling and impregnating machines.

It has been assessed that the addition of polyvinyl alcohol even in small percentages of the order of 0.2-0.3% by weight referred to the weight of the paper, to the concentrated black liquors, causes their behaviour, as an additive for the improvement of the basic qualities of the treated paper, to be enhanced.

Lastly it is to be noted that, as already assessed in the filed tests, the vegetal source of the black liquors must be selected as a function of the mainly desired results.

For instance, whereas the black liquors obtained from multiannual plants by semichemical or soda/ sulfate cooling mainly give place to an improvement of the crushing strength, those obtained from annual plants (straw and the like) by the same cooking treatments mainly give place to an improvement of the bursting strength, whereby the former shall be more advantageous for the treatment of papers to be used for "medium", whereas the latter shall be useful for the "liners".

Lastly the bisulfphite type cooking of multiannual plants gives black liquors qualitatively increasing the crushing strength and the bursting strength without any of the two improvements substantially prevaling with respect to the other.

## Claims

1. A process for making paper, cardboards or paperboards, for a fibre suspension, wherein a paper having a moisture content not greater than 50% is treated with black liquor, characterized in that the black liquor has a solid content from 10% to 50%, the fibres contain at least 20% of waste paper fibres, and the black liquor is added with polyvinyl alcohol.

2. A process according to claim 1, characterized in that the ratio between the content of dry material of the paper and the content of dry materials of the black liquors after concentration is of between 50:10 and 92:10.

3. A process according to claim 2, characterized in that said ratio is of between 50:10 and 80:50.

4. A process according to claim 1, characterized in that a paper containing semichemical pulp is treated in order to increase the crushing strength thereof.

5. A process according to claim 4, characterized in that said semichemical paper has a content of wood pulp not greater than 60%.

6. A process according to claim 1, characterized in that the paper is entirely manufactured from waste paper pulp.

7. A process according to claim 1 to 6, characterized in that the resulting paper is corrugated.

8. A process according to claim 1, characterized in that said concentrated black liquors are added with at least 0.2% by weight, referred to the weight of the paper, of polyvinyl alcohol.

## Patentansprüche

1. Verfahren zur Herstellung von Papier, Karton oder Pappe aus einer faserigen Suspension, in der ein Papier mit einem Feuchtigkeitsgehaltvon nicht mehr also 50% mit schwarzer Lauge behandelt wird, dadurch gekennzeichnet, daß die schwarze Lauge einen Feststoffgehalt von 10% bis 50% hat, die Fasern mindestens 20% von Abfallpapierfasern aufweisen und der schwarzen Lauge Polyvinylalkohol hinzugesetzt wird.

2. Verfahren nach Anspruch 1, dadurch gekennzeichnet, daß das Verhältnis zwischen dem Inhalt von Trockenmaterial des Papieres und dem Inhalt von trockenen Materialien der schwarzen Lauge nach der Konzentration zwischen 50:10 und 92:10 liegt.

3. Verfahren nach Anspruch 2, dadurch gekennzeichnet, daß das Verhältnis zwischen 50:10 und 80:50 liegt.

4. Verfahren nach Anspruch 1, dadurch gekennzeichnet, daß ein Papier, das halbchemischen Zellstoff enthält, behandelt wird zum Erhöhen dessen Druckfestigkeit.

5. Verfahren nach Anspruch 4, dadurch gekennzeichnet, daß das halbchemische Papier einen Gehalt von Holzzellstoff von nicht mehr also 60% hat.

6. Verfahren nach Anspruch 1, dadurch gekennzeichnet, daß das Papier ganz aus Abfallpapierzellstoff hergestellt wird.

7. Verfahren nach einem Ansprüche 1 bis 6, dadurch gekennzeichnet, daß das Papier gewellt ist.

8. Verfahren nach Anspruch 1, dadurch gekennzeichnet, das konzentrierte schwarze Lauge mit mindestens 0,2 Gewichtsprozent, bezogen auf das Gewicht des Papieres, von Polyvinylalkohol hinzugesetzt wird.

## Revendications

1. Procédé de fabrication de papier, carton ou carton ondulé, à partir d'une suspension fibreuse, dans lequel un papier ayant une teneur en humidité qui ne dépasse pas 50% est traité avec une liqueur noire, caractérisé en ce que ladite liqueur noire a une teneur en solide de 10% à 50%, que les fibres contiennent au moins 20% de fibres de papier de recupération, et que les liqueurs noires sont complementées avec de l'alcool polyvinylique.

2. Procédé selon la revendication 1, caractérisé en ce que le rapport entre la teneur en solide du papier et la teneur en solide des liqueurs noires après la concentration est compris entre 50:10 et 92:10.

3. Procédé selon la revendication 2, caractérisé en ce que ledit rapport est compris entre 50:10 et 80:50.

4. Procédé selon la revendication 1, caractérisé en ce qu' on traite un papier contenant pâte semi-chimique pour augmenter sa résistance à l'écrasement.

5. Procédé selon la revendication 4, caractérisé en ce que ledit papier semi-chimique a une teneur en pâte de bois qui ne dépasse pas 60%.

6. Procédé selon la revendication 1, caractérisé en ce que le papier est entièrement fabriqué à partir de pâte de papier de récupération.

7. Procédé selon l'une quelconque des revendications 1 à 6, caractérisé en ce que le papier resultant est ondulé.

8. Procédé selon la revendication 1, caractérisé en ce que lesdites liqueurs noires concentrées son complétées avec au moin 25% en poids, rapporté au poids du papier de l'alcool polyvinylique.
